

## UNITED STATES PATENT OFFICE.

WILLOUGHBY STATHAM SMITH, OF BENCHAMS, NEWTON POPPLEFORD, AND HENRY JOSEPH GARNETT, OF LYMNE, SOLEFIELDS, SEVENOAKS, ENGLAND.

## MAGNETIC ALLOY.

No Drawing. Original application filed January 10, 1924, Serial No. 685,432, and in Great Britain August 25, 1923. Divided and this application filed May 2, 1925. Serial No. 27,594.

This application is a division of our application Ser. No. 685,432, filed January 10, 1924.

This invention relates to the production of alloys possessing a high magnetic permeability especially at low magnetizing forces.

It is well known that it is desirable to add inductance to telegraphic and telephonic cables and this has before been done by 10 wrapping around the core of the cable an iron tape or wire.

Many research workers have been investigating the properties of various alloys, especially those of nickel and iron, with a view to discovering an alloy that should be suitable for this purpose. In our researches we have found that an alloy may be made of nickel, copper and iron, which has a low hysteresis loss with a very high permeability 20 at low magnetizing forces such as those present in telegraphic and telephonic cables.

According to this invention we make an alloy consisting of nickel 73% to 73.75%, iron about 20%, and copper between 4% 25 and 6%.

In order also to increase the electrical resistance of the alloy we preferably add to it a fourth element which may be tungsten, chromium, silicon, vanadium, titanium, molybdenum or aluminium; the amount of this 30 fourth element is small compared to the amount of copper and is preferably less than 1%, since the addition of more than 1% of this fourth element, though increasing the resistance, will impair the permeability 35 of the alloy considerably.

We also preferably include a small amount of manganese to render the alloy more easy 40 to forge; large amounts of manganese may be added to secure an increased electrical resistance.

The following is an example of an alloy made in accordance with this invention.

An alloy consisting of:—

|           | Per cent. |
|-----------|-----------|
| Nickel    | 73.75     |
| Iron      | 20.0      |
| Copper    | 4.5       |
| Manganese | 1.75      |

50 has an electrical resistance of 26 microhms

per cubic centimetre and an initial magnetic permeability of 4800. This alloy is sensitive to heat-treatment and should be annealed by heating to a 55 considerable temperature and then cooled. This may conveniently be done by passing a wire or tape formed of the alloy through a tube heated electrically and allowing the wire or tape to cool rapidly as it issues from 60 the tube.

If the correct temperature has not been used the magnetic properties will not be fully developed.

The annealing may be adjusted to give 65 either:—

(a) Maximum initial permeability, or (b) maximum permeability at magnetic saturation, and (c) low or high fields for 70 magnetic saturation.

## Example.

The above mentioned alloy—

(a) Annealed at 850° C. and air cooled; initial permeability, 4800; saturation permeability, 12300; field for magnetic saturation, .35 c. g. s. units.

(b) Annealed at 830° C. and cooled more slowly; initial permeability, 4700; saturation permeability, 30000; field for magnetic 80 saturation, .10 c. g. s. units.

Moreover, when correctly annealed for high initial permeability, the alloys have low hysteresis losses varying from 50 to 150 ergs per cubic centimetre with a maximum 85 field of .25 c. g. s. units.

What we claim is:—

1. An alloy consisting of nickel 73.75%, iron 20%, copper 4.5% and manganese 1.75%.

2. An alloy consisting of nickel from 73 to 74%, iron 20 to 21%, copper 4.5 to 5.4%, manganese 1.5 to 2%, and another element adapted to increase the electrical resistance of the alloy.

In testimony that we claim the foregoing as our invention we have signed our names this twenty-first day of April, 1925.

WILLOUGHBY STATHAM SMITH.  
HENRY JOSEPH GARNETT.